

1

3,223,524

PROCESS FOR THE PRODUCTION OF PLANO-GRAPHIC PRINTING PLATES HAVING AN ALUMINUM SUPPORT

Anita von König, Leverkusen, Germany, assignor to Agfa Aktiengesellschaft, Leverkusen, Germany, a corporation of Germany  
No Drawing. Filed Sept. 26, 1960, Ser. No. 58,181  
5 Claims. (Cl. 96—29)

The invention relates to a method for improving planographic printing plates having an aluminium support.

It is known that photographically produced silver images can be transformed into heavy metal and/or silver salt images by oxidation. The resulting images can be reacted with an organic compound containing an SH-, SeH- or NH-group to produce sparingly soluble salt-like compounds which take up greasy printing inks.

It is also known that photographic silver images can be deposited by the silver salt diffusion process on to unprepared aluminium plates having a rough surface and which are suitable for planographic printing. The silver images can be made water-repellent by treating them with an organic compound which is capable of being adsorbed by metallic silver so as to render the images capable of taking up greasy printing inks. In this way planographic printing plates are obtained. Suitable organic compounds which are capable of being adsorbed by metallic silver described in the copending application Serial No. 730,259, now U.S. Patent 3,083,097, are 2,5-dimercapto-1,3,4-thiodiazole, 5-mercaptop-3-phenyl-1,3,4-thiodiazolethione-2,5 - mercaptotetrazole, 1-phenyl-5-mercaptotetrazole, 3-mercaptop-1,2,4-triazole, 1-phenyl-3-mercaptop-1,2,4-triazole, 2,4,6-trimercapto-1,3,5-triazine, 2-mercaptop-4,5-dimethyl-6-oxyprymidine, 6 - mercaptopyrimidine, tetraethyl thiuram disulphide, thiourea, phenyl thiourea, phenyl thiosemicarbazide, diphenyl thiosemicarbazide, diphenyl thiocarbazone, diphenyl carbazide and compounds of the general formula



wherein R represents an alkyl radical, X represents an NH group or an oxygen or sulphur atom and Y represents an oxygen or sulphur atom.

The aforementioned compounds, however, do not in many cases impart a sufficient water-repellent character to the silver images.

Either the color absorption is too small on account of the water-repelling effect being too weak, or in certain cases where the color absorption is good the silver images which have been made water-repellent are unstable with respect to atmospheric influences and with respect to dilute phosphoric acid. It is essential that the silver images which have been made water-repellent have a high resistance to atmospheric influences since the planographic printing plates have to be stored in the printing works for several hours or even days. The planographic printing plates must also be resistant to dilute phosphoric acid, because the printing inks and moistening mechanisms of the printing machines and also the sponges used for rubbing down the fixing contain phosphoric acid.

2

For practical reasons it is preferable if the organic compounds employed for the purpose of making the silver images water-repellent are soluble or are capable of being suspended in the fixing solutions normally employed in planographic printing. Especially suitable are aqueous solutions of gum arabic, polyvinyl alcohol and carboxymethyl cellulose, which are adjusted to a pH of from 4 to 6 by means of phosphoric acid or a phosphate. This adjustment of the pH is effected in the absence of an organic solvent, since organic solvents dissolve the printing inks.

It has now been found that silver images which have been produced on aluminium plates by the silver salt diffusion process can be rendered capable of taking up ink satisfactorily if there is used for producing the water-repellent effect a solution or suspension containing a derivative of 2-mercaptop-1,3,4-thiodiazole which contains at least two mercapto groups and at least two 1,3,4-thiodiazole radicals bonded by way of an organic radical. Especially suitable are compounds of the general formula



wherein Z stands for (I) alkylene with 1 to 6 carbon atoms, (II) —S.A.S—, wherein A is (1) a bivalent hydrocarbon radical, preferably an alkylene group having 1 to 10 carbon atoms or an aralkylene group, such as xylylene which is substituted in the benzene nucleus by aliphatic radicals, or (2) an alkylene group interrupted by hetero atoms, preferably oxygen atoms, preferably a group having the structure



40 wherein n is an integer, preferably from 1 to 5, and m is an integer from 2 to 4, or (III) —NH.B.NH—, wherein B stands for alkylene with 4 to 10 carbon atoms, cycloalkylene or arylene.

45 The compounds of the type



50 are described in Chemical Abstracts 1960, 1502b, respectively Journal of Chemical Society (Jap.), Pure Chemical Section 78 (1957), 1588 to 1591. The melting points of some of said compounds are given in the 55 following Table 1:

TABLE 1

| Compound | Number of $\text{CH}_2$ -groups | Melting point, deg. |
|----------|---------------------------------|---------------------|
| I.....   | n=0                             | 292-293             |
| II.....  | n=2                             | 280-283             |
| III..... | n=4                             | 195                 |

The compounds of the type



can be prepared as follows:

2 mols of 2,5-dimercapto-1,3,4-thiodiazole are dissolved in a solution of 2 mols of sodium or potassium hydroxide in 1200 cc. of aqueous alcohol (85% by volume). 1 mol of an  $\alpha,\omega$ -dihalogenoalkane is added to this solution. The solution is boiled for 2 to 6 hours under reflux and, after cooling, the precipitated product is suction-filtered and washed free from halogen. The yield is 85 to 95%. The product is purified by recrystallization from alcohol or by being repeatedly dissolved and crystallized. The melting points of some of the compounds prepared in this way are given in the following Table 2:

TABLE 2

| Compound | -A-                                                                      | Melting point, deg. |
|----------|--------------------------------------------------------------------------|---------------------|
| IV       | $-\text{CH}_2-$                                                          | 174-176             |
| V        | $-(\text{CH}_2)_2-$                                                      | 214-216             |
| VI       | $-(\text{CH}_2)_3-$                                                      | 162-163             |
| VII      | $-(\text{CH}_2)_4-$                                                      | 191-193             |
| VIII     | $-(\text{CH}_2)_5-$                                                      | 162-163             |
| IX       | $-(\text{CH}_2)_6-$                                                      | 145-147             |
| X        | $-(\text{CH}_2)_{10}-$                                                   | 131-132             |
| XI       | $-\text{CH}_2-\text{C}_6\text{H}_4-\text{CH}_2-$                         | 223                 |
| XII      | $-\text{CH}_2-\text{C}_6\text{H}_3(\text{CH}_3)_2-\text{CH}_2-$          | 220                 |
| XIII     | $-\text{CH}_2\text{CH}_2\text{OCH}_2\text{CH}_2-$                        | 80                  |
| XIV      | $-\text{CH}_2\text{CH}_2\text{OCH}_2\text{CH}_2\text{OCH}_2\text{CH}_2-$ | 105-106             |

A compound of the type



can be prepared as follows:

65.5 g. (0.25 mol) of 4,4'-(1,4-cyclohexylene)-dithiosemicarbazide are dissolved in 600 cm.<sup>3</sup> dimethyl formamide. While stirring 70 cm.<sup>3</sup> of carbon disulphide are added dropwise to this solution at room temperature. The solution is heated to 65° C. within 90 minutes and kept at this temperature for 20 hours until the development of hydrogen sulphide is finished. The product is precipitated by stirring the reaction mixture into aqueous hydrogen chloride which is cooled with ice. The precipitated product is suction-filtered and washed free from halogen. The raw material is purified by reprecipitation.

The yield is 48 g. with a melting point of 273°. The melting points of some of the compounds prepared in this way are given in Table 3

TABLE 3

| Compound | -B-                                              | Melting point, deg. |
|----------|--------------------------------------------------|---------------------|
| XV       | $-(\text{CH}_2)_6-$                              | 198-199             |
| XVI      | $\text{C}_6\text{H}_5-$                          | 271-273             |
| XVII     | $\text{C}_6\text{H}_4-$                          | 299-300             |
| XVIII    | $-\text{CH}_2-\text{C}_6\text{H}_4-\text{CH}_2-$ |                     |
| XIX      | $\text{C}_6\text{H}_4-\text{C}_6\text{H}_4-$     |                     |

The compounds are suspended, with the aid of emulsifiers, in an aqueous alkali solution or in the fixing solutions normally employed in planographic printing. The compounds are generally employed in an amount of from 5 to 20 g./l. The silver images produced in known manner on an aluminium foil having a rough surface by the silver salt diffusion process are made water-repellent by coating them with the aforementioned solutions or suspensions.

It is also possible to use a solution of one of the aforementioned compounds and the acid fixing solution successively in separate working steps.

It is, however, more desirable to combine the compounds with a fixing solution known as per se in connection with planographic printing using aluminium plates, for example with an aqueous solution of gum arabic, polyvinyl alcohol, carboxymethyl cellulose, derivatives of alginic acid such as alkaline salts, amides and esters and caragheenate (extracts of red seaweed, described in Melland Textilbrichte 1960, pages 596 to 600 and 861 to 865), which is adjusted by means of phosphoric acid or a phosphate to a pH of from 4 to 6. After the silver image has been made water-repellent and the plate has been fixed, which operations take place simultaneously, the printing ink is applied to the foil either by rubbing or rolling by hand or by the printing machine. The printing portions are distinguished by a high bonding strength for greasy printing ink. About 5000 satisfactory prints can be produced.

In order to produce stable suspensions of the compounds in the acid fixing solutions, the compounds must be emulsified by means of emulsifiers, preferably anionic-active emulsifiers. Suitable emulsifiers and emulsifying auxiliaries are given in Table 4.

TABLE 4

| Emulsifier | Name                   | Constitution                                     | Manufacturer               |
|------------|------------------------|--------------------------------------------------|----------------------------|
| 1          | Monopolbrillantöl      | Sulphonate castor Oil                            | Stockhausen & Co. Krefeld. |
| 2          | Teepol                 | Sec. alkyl Sulphate                              | Shell.                     |
| 3          | Hostapar A             | Sodium oleoylsarcosinate                         | Hoechster Farbwerke.       |
| 4          | Emulgator 0            | Acid diethylamino oleate                         | Farbenfabriken Bayer A.G.  |
| 5          | Tamol NNO              | Dinaphthyl methane sulphonate                    | Bad. Anilin u.Soda-Fabrik. |
| 6          | Humectol C             | Dibutylamide of sulphonated ricinoleic acid.     | Casella-Farbwerke.         |
| 7          | Polyglycol P 400       |                                                  | Hoechster Farbwerke.       |
| 8          | Texapon Z (high conc.) | Sulphate of coconut fatty alcohol                | Dehydag.                   |
| 9          | Polystate              | Mono- and distearate of polyethylene glycol 300. | SOG EP.                    |
| 10         | Emulgator NP 10        |                                                  | Farbenfabriken             |
| 11         | Tween 40               | Polyethylene sorbitane monopalmitate             | Bayer A.G.                 |
| 12         | Emulgator 157          | Propylenglycol mono- and distearate              | Atlas-Goldschmidt G.m.b.H. |



wherein Z stands for a bivalent member selected from the group consisting of (I) alkylene having up to 6 carbon atoms; (II) —SAS, wherein A is a member selected from the group consisting of alkylene of 1-10 carbon atoms, phenylalkylene,  $[(\text{CH}_2)_m-(\text{CH}_2)_n]_n$  wherein  $m$  is 2-4 and  $n$  is 1-4; and (III) —NH—B—NH— wherein B is a member selected from the group consisting of alkylene of 4-10 carbon atoms, cyclohexylene, phenylene, diphenylene, and phenylalkylene.

2. A process for producing planographic printing plates consisting in developing an imagewise exposed silver halide emulsion layer while in contact with an aluminum plate in a silver halide developer solution containing a silver halide solvent for dissolving silver halide from the unexposed areas of said silver halide emulsion layer, transferring the dissolved unexposed silver halide to said aluminum plate and reducing the dissolved silver halide on said aluminum plate to obtain a corresponding silver image, characterized in thereafter contacting said silver image directly with a hydrophobing amount of a 2-mercapto-1,3,4-thiodiazole having the formula



wherein Z stands for a bivalent member selected from the group consisting of (I) alkylene having up to 6 carbon atoms; (II) —SAS, wherein A is a member selected from the group consisting of alkylene of 1-10 carbon atoms, phenylalkylene,  $[(\text{CH}_2)_m-\text{O}-(\text{CH}_2)_n]_n$  wherein  $m$  is 2-4 and  $n$  is 1-5; and (III)



wherein B is a member selected from the group consisting of alkylene of 4-10 carbon atoms, cyclohexylene, phenylene, diphenylene, and phenylalkylene.

3. The process of claim 2, wherein the silver image is

treated with a dispersion containing, in addition to the thiodiazole at least one product selected from the class consisting of carboxymethyl cellulose, polyvinyl alcohol, gum arabic, alginic acid, alkali salts of alginic acid, amides of alginic acid, esters of alginic acid and carageenates; and a member selected from the class consisting of phosphoric acid and acid water-soluble phosphates.

4. The process of claim 2, wherein the silver images are treated with a dispersion which has been prepared with the aid of emulsifiers and emulsifying auxiliaries.

5. The process of claim 2, wherein the silver image is treated with a dispersion containing the thiodiazole derivative and additionally an organic hydrophilic film-forming product which is soluble in said dispersion, and a member selected from the class consisting of phosphoric acid and acid water-soluble acid phosphates.

#### References Cited by the Examiner

##### UNITED STATES PATENTS

|           |         |                |       |           |
|-----------|---------|----------------|-------|-----------|
| 2,184,288 | 12/1939 | Dangelmajer    | ----- | 96-33     |
| 2,352,014 | 6/1944  | Rott           | ----- | 96-29     |
| 2,514,650 | 7/1950  | Knott et al.   | ----- | 96-52     |
| 2,685,588 | 8/1954  | Goshorn et al. | ----- | 260-302   |
| 2,891,961 | 6/1959  | Turner et al.  | ----- | 260-306.8 |
| 3,083,097 | 3/1963  | Lassig et al.  | ----- | 96-29     |

##### FOREIGN PATENTS

|         |         |                |
|---------|---------|----------------|
| 572,336 | 4/1959  | Belgium.       |
| 582,160 | 3/1960  | Belgium.       |
| 582,161 | 3/1960  | Belgium.       |
| 760,181 | 10/1956 | Great Britain. |

##### OTHER REFERENCES

Chemical Abstracts 54, 1502d (1960).

NORMAN G. TORCHIN, Primary Examiner.

PHILIP E. MANGAN, Examiner.